

G. G. CARVER,  
WOOD IMPREGNATION,  
APPLICATION FILED MAY 20, 1915.

1,256,200.

Patented Feb. 12, 1918.

FIG. 1



FIG. 6



FIG. 3



FIG. 5



FIG. 4



FIG. 7



FIG. 2



FIG. II



FIG. 8



Witnesses  
glady Jameson  
C. H. Bauch

By

George G. Carver  
Geo. E. Kirk

Attorney



FIG. 10  
Inventor

# UNITED STATES PATENT OFFICE.

GEORGE G. CARVER, OF TOLEDO, OHIO, ASSIGNOR TO THE JENNISON-WRIGHT COMPANY,  
OF TOLEDO, OHIO, A CORPORATION OF OHIO.

## WOOD IMPREGNATION.

1,256,200.

Specification of Letters Patent. Patented Feb. 12, 1918.

Application filed May 20, 1915. Serial No. 28,273.

To all whom it may concern:

Be it known that I, GEORGE G. CARVER, a citizen of the United States of America, residing at Toledo, Lucas county, Ohio, have 5 invented new and useful Wood Impregnation, of which the following is a specification.

This invention relates to incorporation in connection with a porous, cellular or normally interstice carrying material of additional material.

This invention has utility in charging wood, especially for antisepticizing and waterproofing, thereby acting as a preservative 15 and offering greater resistance against weather attacks when the material is used for railroad ties, piles, poles, paving blocks, etc.

Referring to the drawings:

20 Figure 1 is a greatly enlarged cross section of an interstice carrying material, wood;

Fig. 2 is a view at right angles to the plane of the showing in Fig. 1, showing the general direction of the pores, cells or interstices;

25 Fig. 3 is a view similar to Fig. 1, indicating the penetration for initially fully charging the wood, say with an impregnating solution or waterproofing liquid, as hot coal tar or creosote;

Fig. 4 is a fragmentary section longitudinally of the interstices showing irregular superficial impregnation as developed initially;

30 Fig. 5 is a view similar to Fig. 1, indicating uniform cell coating or interstice wall painting produced in connection with compressible fluid interstice clearing or penetration assisting treatment initially;

Fig. 6 is a view at right angles to the 40 plane of the showing in Fig. 5, showing the uniform penetration of the interstice coating or wood antisepticizing treatment;

Fig. 7 is a view similar to Fig. 1, indicating uniform full charging of the initially 45 interstice cleared wood, say of Fig. 5;

Fig. 8 is a view at right angles to the plane of the showing in Fig. 7, showing the uniform penetration of the full charge longitudinally of the interstices;

50 Fig. 9 is a view similar to Fig. 1, showing the initially opened and coated interstices and the superficially sealed or fully charged treatment of the wood to a less penetration extent than is shown in Fig. 7;

55 Fig. 10 is a view in fragmentary section

longitudinally of the wood pores or interstices, showing wood interiorly fully coated and superficially fully charged, with the penetration to a less complete extent than the showing in Fig. 8; and 60

Fig. 11 is a perspective view of a piece of treated material in the form of a wood paving block.

The interstice carrying material, as wood, may have the interstices 1 of the spring or 65 rapid growth periods, and more closely walled interstices 2 of the summer or slower growth period (Figs. 1, 2).

Notwithstanding the porosity of woods, the interstices naturally vary widely in the 70 resistance to penetration and more particularly by heavy fluids, as waterproofing liquids of the hydrocarbon series, even though heated. Submerging the wood in hot oil or incompressible fluid and subjecting 75 to pressure may produce the irregular superficial penetration in impregnating the open cells 3 and the smaller cells 4 (Figs. 3, 4).

To overcome these irregularities, and 80 thereby make more certain the production of a reliably impregnated product to withstand weathering attacks, the wood to be treated is subjected to initial compressible fluid or gaseous pressure, say by placing the mate-

rial in a treating vessel and pumping air thereinto to the desired number of atmospheres which from the nature of the wood and its particular use may seem proper.

For paving blocks, a pressure of three to 85 five atmospheres may be used to advantage as the timber may be impervious or seasoned. This action should compress the readily

penetrating gas into the most remote and small interstices, tending to rupture thin interstice walls interfering with the penetration of the uniform compression throughout the wood mass. While still carrying this compressible charge, the blocks may be sub-

merged in a coating or impregnating solution, say hot creosote oil and the pressure then run up to say ten atmospheres. This liquid will enter the interstices opened by the compressed air. With temperature and pressure constant for a while, uniform permeation is assisted. 95

Lowering the pressure say to 20 inches of mercury and drawing off of the liquid allows the compressed gas in the timber to expel uniformly a considerable portion of the 100 110

oil which entered the timber. The result is a wood in which the interstices are uniformly thinly coated on their walls, and the interstices cleared uniformly by the outflowing of the compressed air. The spring interstices 5 and smaller summer interstices 6 (Figs. 5, 6) are receptacles rendered uniformly aseptic.

With the interstices thus prepared for sealing or fully charging, the wood may be resubmerged, say in hot oil, which may be at a temperature of say 150° F. in this instance and in the initial submerging. Again the pressure is raised, say to three to five atmospheres, resulting in a uniform impregnation of the interstices 7, 8 (Figs. 7, 8), permitting a maximum and uniform charge even in widely differing timbers and woods normally resisting penetration.

Instead of rendering antiseptic and fully charging in the waterproofing material to procure a maximum impregnation, a superior antiseptic and sealed or superficially waterproofed material may be produced by subjecting to a less strenuous resubmerging pressure treatment. There is then the effective superficial sealing of the interstices 9, 10, with the interior thinly coated and antiseptic interstices 5, 6, affording space to take care of expansion and weathering penetration of the fully charged superficial interstices.

The treated material or wood block 11 (Fig. 11), is dependable uniformly as to its exposed surfaces, for notwithstanding the natural variation in interstitial form, due to growth conditions and soil, as well as weather and other changes causing continual departures from uniformity, the highly penetrable compressed air, has provided communication between the interstices. The hydraulic pressure of a liquid on the compressed air has increased the compression and rupturing action of these two fluids. In the treatment the blowing out of the compressed air upon release of pressure thinly paints or coats the timber cells in a most thorough manner and leaves the passages open, and open uniformly superficially for effective full charging or superficial but still true sealing, as may be desired.

What is claimed and it is desired to secure by Letters Patent is:

1. The process of providing sealed internal expansion space in the treating of wood

comprising, first, coating the cell walls of the wood by submerging said wood in a preserving liquid, subjecting said submerged wood to pressure, lowering the pressure and removing the excess submerging liquid, and second, superficially fully impregnating the wood by re-submerging the wood in an impregnating liquid and applying pressure thereto of a less amount than in the preceding submerging to provide space in the wood interior of this second treatment for the second treatment to expand thereinto.

2. The process of providing sealed internal expansion space in treating wood comprising, first, coating the cell walls by subjecting the wood to gas pressure and with the gas still entrained in the wood, submerging said wood in a preserving liquid, subjecting said submerged wood to increased pressure, lowering the pressure and removing the excess submerging liquid expressed from the wood by the expanding gas due to the lowering of such pressure, and, second, superficially fully impregnating the wood with a substance for effective waterproof sealing of the unfilled interior coated walls that expansion of the sealing substance may occur thereinto.

3. The method of providing sealed internal expansion space in treating wood comprising, first, coating the cell walls by subjecting the wood to gas pressure and without relieving the gas pressure, subjecting the same to a bath of a preserving substance under a higher pressure than the gas pressure, withdrawing the surplus substance, and immediately subjecting the wood to a partial vacuum thereby extracting a portion of the preserving substance from the wood, and, second, superficially fully impregnating the wood for effective water-proofing by submerging the wood in an impregnating liquid, subjecting said submerged wood to pressure less than the pressure employed in the first treatment whereby the exterior cells may be sealed and expansion of the sealing liquid may occur into the internal coated cells.

In testimony whereof I affix my signature in the presence of two witnesses.

GEO. G. CARVER.

Witnesses:

A. E. MURBACH,  
R. F. SCHNEIDER.